# EUROPEAN PATENT SPECIFICATION

(11) **EP 0 475 101 B1**
(45) Date of publication and mention of the grant of the patent: **13.12.1995**
(21) Application number: 91113667.9
(22) Date of filing: 14.08.1991
(51) Int. Cl.: C22C 1/00

(54) **High strength aluminum-based alloys**
Hochfeste Legierungen auf Aluminiumbasis
Alliages à base d'aluminium, à haute résistance

(30) Priority: 14.08.1990 JP 213755/90
(43) Date of publication of application: 18.03.1992
(73) Proprietor: YKK CORPORATION, Chiyoda-ku, Tokyo (JP)
(72) Inventor: Nagahora, Junichi, Yokohama-shi, Kanagawa (JP); Terabayashi, Takeshi, Shimoniikawa-gun, Toyama (JP); Kawanishi, Makoto, Kurobe-shi, Toyama (JP); Taketani, Katsuyuki, Kawasaki-shi, Kanagawa (JP)
(74) Representative: Patentanwälte Leinweber & Zimmermann

(56) References cited:
- EP-A- 0 136 508
- EP-A- 0 339 676
- DE-A- 3 524 276

## Description

### BACKGROUND OF THE INVENTION

### 1. Field of the Invention

The present invention relates to aluminum-based alloys having a high strength together with a high hardness, high wear resistance, high heat resistance and superior toughness.

### 2. Description of the Prior Art

Aluminum-based alloys having a high strength and a high heat resistance have heretofore been produced by a liquid quenching method. Ultra fine grained Al based powder alloys having the general formula AlₓMe_{y}Ce_{z} (Me=Fe, Mo, Co or Ni) are disclosed in e.g. in DE-A-3 524 276. Moreover, the document EP-A-0 136 508 discloses rapidly solidified aluminium based alloys of the general formula Al_{bal}FeₐX_{b} (X = Zn, Co, Ni, Cr, Mo, V, Zr, Ti,Y, Si and Ce) comprising uniformly dispersed intermetallic phase precipitates of less than about 100 nm, preferably less than 20 nm. For instance, Japanese Patent Application Laid-Open No. 1-275732 & EP-A-0339676 discloses aluminum-based alloys produced by the liquid quenching method and the aluminum-based alloys have an amorphous or fine crystalline structure and are superior alloys characterized by having an advantageous combination of properties of high strength, high heat resistance and high corrosion resistance.

The aluminum-based alloys disclosed in the above Japanese Patent Application Laid-Open No. 1-275732 are superior alloys having a high strength, high heat resistance and high corrosion resistance and also exhibit a high degree of processability as high strength materials. However, the aluminum-based alloys should still be improved in their toughness for applications as materials where a high toughness is required.

In view of the foregoing, it is an object of the present invention to provide materials having a superior toughness, while retaining an adequate strength, and, thereby, are useful in structural component applications where a high reliability is required.

The present invention provides a high strength aluminum-based alloy having a composition consisting of the general formula (I) AlₐM_{b}Ln_{c} or the general formula (II) AlₐM_{b}X_{d}Ln_{c},
wherein:
M is at least one metal element selected from the group consisting of Co, Ni, and Cu;
X is at least one metal element selected from the group consisting of V, Mn, Fe, Mo, Ti and Zr;
Ln is at least one element selected from the group consisting of Y, rare earth elements and Mm (misch metal), which is a composite of rare earth elements; and
a, b, c and d are, in atomic percentage,
75 ≦ a ≦ 97, 0.5 ≦ b ≦ 15, 0.5 ≦ c ≦ 10 and 0.5 ≦ d ≦ 3.5,
the alloy being composed of an aluminum matrix or an aluminum supersaturated solid solution matrix having an average crystal grain size of from 0.1 to 80 »m and containing therein a uniform dispersion of metastable or stable phase particles composed of intermetallic compounds, which are formed between the host element (matrix element) and the above-mentioned alloying elements and/or between the alloying elements, the intermetallic compounds having an average particle size of 10 to 500 nm.

### BRIEF DESCRIPTION OF THE DRAWINGS

FIG. 1 shows a schematic illustration of a single-roller melt spinning apparatus employed to prepare a thin ribbon by rapidly quenching and solidifying alloys of the present invention.

FIG. 2 is a graph showing the test results of alloys of the present invention.

### DETAILED DESCRIPTION OF THE PREFERRED EMBODIMENTS

The aluminum-based alloys of the present invention can be obtained by rapidly solidifying a melt of the alloy having the composition as specified above by employing liquid quenching techniques. The liquid quenching techniques are methods for rapidly cooling a molten alloy and, particularly, single-roller melt-spinning, twin-roller melt-spinning and in-rotating-water melt-spinning are effective. In these techniques, a cooling rate of about 10⁴ to 10⁶ K/sec can be obtained. In order to produce thin ribbon materials by single-roller melt-spinning technique or twin-roller melt-spinning, the molten alloy is ejected from the bore of a nozzle onto a roll of, for example, copper or steel, with a diameter of about 30 - 300 mm, which is rotating at a constant rate within the range of about 300 - 10000 rpm. Thus, various thin ribbon materials with a width of about 1 - 300 mm and a thickness of about 5 - 500 »m can be readily obtained. Alternatively, in order to produce wire materials by in-rotating-water melt-spinning, a jet of the molten alloy is directed, under application of a back pressure of argon gas, through a nozzle into a liquid refrigerant layer having a depth of about 1 to 10 cm and which is held by centrifugal force in a drum rotating at a rate of about 50 to 500 rpm. In such a manner, fine wire materials can be readily obtained. In this process, the angle between the molten alloy ejecting from the nozzle and the liquid refrigerant surface is preferably in the range of about 60° to 90° and the relative velocity ratio of the ejected molten alloy to the liquid refrigerant surface is preferably in the range of about 0.7 to 0.9.

Besides the above processes, the alloy of the present invention can also be obtained in the form of a thin film by a sputtering process. Further, rapidly solidified powder of the alloy composition of the present invention can be obtained by various atomizing processes (for example, high pressure gas atomizing) or spray process.

Whether the resultant rapidly solidified aluminum alloys have an average crystal grain size of 0.1 to 80 »m can be examined using a transmission electron microscope. In detail, the grain sizes of individual crystals can be measured from the contrast resulting from the difference in crystal orientation of the respective crystals which contrast is observed in a bright-field of about 1000 to 100,000 magnifications. When the individual crystals can not be distinctly observed in the bright-field, they can be examined through observation in a dark-field of a certain electron diffraction spot. The average particle size of intermetallic compounds can be examined in the same way. The presence of intermetallic compounds can be confirmed through an ordinary electron diffraction. The intermetallic compounds can be easily distinguished from an aluminum matrix in the electron diffraction image.

As previously described, the alloys of the present invention can be obtained by the above-mentioned single-roller melt-spinning process, twin-roller melt spinning process, in-rotating-water melt spinning process, sputtering process, various atomizing processes, spraying process, mechanical alloying process, mechanical grinding process, etc. It is possible to control the average sizes of crystal grains and intermetallic compound particles of the resultant alloys by appropriately varying the processing conditions according to the need.

Further, depending on the composition, alloys having an amorphous structure can be obtained but the amorphous structure decomposes into a crystalline structure when being heated to a certain temperature or higher. The alloys of the present invention can also be obtained by the thermal decomposition of the amorphous structure and, in this decomposition process, the average grain size can be controlled within the range of the present invention by properly adjusting the heating conditions.

In the aluminum-based alloys represented by the general formula (I) or (II), a, b, c and d are limited to the atomic percentages ranging from 75 to 97%, 0.5 to 15%, 0.5 to 10% and 0.5 to 3.5%, respectively. The reason for these limitations is that when a, b, c and d are outside the specified ranges, the resultant alloys become brittle and toughness and high strength can not be achieved. Consequently, alloys having properties contemplated by the present invention can not be obtained by industrial rapid quenching processes employing a liquid quenching or the like.

The M element is at least one metal element selected from the group consisting of Co, Ni and Cu. Although the M element has a relatively poor diffusion tendency in an aluminum matrix, it forms various stable or metastable fine intermetallic compounds in coexistence with the Ln element. The resultant intermetallic compounds are finely dispersed throughout the aluminum matrix, thereby effectively preventing an extraordinary grain coarsening as well as strengthening the matrix. Consequently, the M element considerably improves the hardness and strength of the alloys and stabilizes fine crystalline phases both at room temperature and at an elevated temperature, thereby providing an improved heat resistance.

The X element is at least one metal element selected from the group consisting of V, Mn, Fe, Zr, Ti and Mo. Although the X element exhibits a relatively low diffusion tendency in an aluminum matrix, it has an effect in retaining the room temperature hardness and strength up to elevated temperatures. Further, addition of the X element in amounts of 0.5 to 3.5 atomic percent is advantageous, especially when processed materials are produced by a hot plastic forming, because the X element addition provides ductility.

The Ln element is at least one element selected from the group consisting of Y, rare earth elements and Mm (misch metal). The Ln element also has a low diffusion ability in an aluminum matrix but, when it is contained in coexistence with the foregoing M element, it forms stable intermetallic compounds and makes a great contribution to stabilization of the fine crystalline structure.

Within the alloy compositional ranges of the present invention, an amorphous phase or an average crystal grain size of less than 0.1 »m can also be obtained. However, in such a case, the ductility (i.e., toughness) is not sufficient for the intended use of the present invention, although the strength is high. In order to achieve the desired ductility, i.e., at least 0.5% tensile elongation, an average crystal grain size of 0.1 »m or greater is essential.

Further, an average crystal grain size exceeding 80 »m may be obtained by employing an excessively reduced cooling-rate or an excessively increased processing temperature for the thermal decomposition, but, in such conditions, the strength will be drastically reduced. Therefore, the object of the present invention can not be achieved.

Proper choice of the heating conditions provides an average crystal grain size controlled within the range contemplated by the present invention.

In the present invention, the particle size of intermetallic compounds is limited to the range of 10 to 500 nm because when the size is outside the specified range, the intermetallic compounds do not act as a matrix strengthening component. In detail, an excessively increased cooling rate or an inadequate processing temperature for the thermal decomposition results in intermetallic compounds having a particle size of less than 10 nm. Such fine intermetallic compounds have no effect in strengthening the aluminum matrix. Further, when the intermetallic compounds excessively dissolve in the matrix as a solid solution, a problem of brittleness may arise. On the other hand, when the cooling rate is excessively reduced or the processing temperature of the thermal decomposition is too high, the resultant intermetallic compounds have an average particle size exceeding 500 nm and produce no strengthening effect. That is, the dispersed particles become too large and it does not exhibit any strengthening effect. Within the above-specified range, greatly improved Young's modulus, high-temperature strength and fatigue strength can be obtained.

As set forth above, in the production of the alloys of the invention, proper choice of the production conditions makes it possible to control the crystal grain size and the average particle size of intermetallic compounds. Therefore, when strength is important, the average crystal grain size and the intermetallic compound particle size are controlled to small sizes. Alternatively, when ductility is required, the crystal grain size and the intermetallic compound particle size are controlled to large sizes. In such a manner, the properties can be controlled according to the purposes.

When the crystal grain size is controlled within the range of 0.1 to 10 »m, properties desirable as superplastic forming materials can also be obtained.

The alloys of the present invention can be obtained in the form of ribbons, thin strips or powders and can be readily processed into bulk materials using hot plastic forming processes, such as extrusion, press forming or forging, within the temperature range of one-fifth (1/5) to one half (1/2) the melting point of the alloys. Also, bulk materials can also be readily obtained from the alloys having an amorphous structure or a supersaturated solid solution structure by appropriately controlling the powder consolidation conditions. The alloys of the present invention exhibit superior properties as extremely tough and strong alloys and, thus, are especially useful as highly reliable structural materials.

Hereinafter, the present invention will be explained in more detail with reference to the following examples.

### Examples

Molten alloy 3, having a predetermined composition, was prepared using a high-frequency melting furnace and charged into a quartz tube 1 having a small opening 5 (diameter: 0.5 mm) at the tip thereof, as shown in FIG. 1. After being heated to melt the alloy 3, the quartz tube 1 was disposed right above a copper roll 2. Then, the molten alloy 3 contained in the quartz tube 1 was ejected from the small opening 5 of the quartz tube 1 under the application of an argon gas pressure of 0.7 kg/cm² and brought into contact with the surface of the copper roll 2 rapidly rotating at a rate of 1,000 rpm. The molten alloy 3 was rapidly quenched and solidified into an alloy thin ribbon 4.

According to the processing conditions as described above, 14 different alloy thin ribbons (width: 1 mm, thickness: 20 »m) having the compositions (by at.%) as shown in Table 1 were obtained and test specimens were prepared. The average crystal grain size of each test specimen was measured through observation by transmission electron microscopy (TEM). The measurement results showed that all of the test specimens were composed of a crystalline matrix having an average crystal grain size of 0.1 to 60 »m and containing intermetallic compounds having an average particle size of 10 to 50 nm therein. It was found that no amorphous phase was contained in the test specimens.

The mechanical properties measured by a tensile test at room temperature, and microVickers hardness (under a load of 50g) are also set out in Table 1.

**Table 1**

| Composition (at. %) | | Hv(DPN) | ^{σ}max^{(MPa)} | ε(%) |
|---|---|---|---|---|
| 1 | Al₈₅Ni₅Fe₂Y₈ | 275 | 920 | 2.5 |
| 2 | Al₈₇Ni₈Y₅ | 273 | 890 | 2.7 |
| 3 | Al₉₀Ni₅La₅ | 264 | 890 | 2.6 |
| 4 | Al₉₂Ni₅V₁Mm₂ | 297 | 910 | 1.7 |
| 5 | Al₈₈Fe₂Co₂Ce₈ | 312 | 915 | 2.2 |
| 6 | Al₈₈Fe₂Zr₂Mm₈ | 305 | 927 | 1.8 |
| 7 | Al₈₈Cu₄Ni₂Mm₆ | 267 | 945 | 1.7 |
| 8 | Al₉₂Cu₄Ni₂Y₂ | 256 | 875 | 2.8 |
| 9 | Al₉₀Co₄Ni₂Y₄ | 256 | 890 | 1.7 |
| 10 | Al₈₇Co₄Ti₂Mm₇ | 275 | 920 | 1.6 |
| 11 | Al₉₀Ni₆Zr₁Mm₃ | 273 | 930 | 2.9 |
| 12 | Al₉₀Ni₈Zr_{0.5}Mm_{1.5} | 278 | 928 | 2.3 |
| 13 | Al_{89.5}Ni₈Zr₁Fe_{0.5}Mm₁ | 273 | 912 | 2.6 |
| Remark: Hv(DPN): microVickers hardness ^{σ}max^{(MPa)}: ultimate tensile strength ε(%): Tensile elongation | | | | |

All of the samples were found to be superior alloys having an elongation of at least 1.6% coupled with a strength of at least 875 MPa.

Next, alloy powders, having an average particle size of not greater than 45 »m and consisting of an amorphous phase, were prepared by an atomizing process with a high-pressure gas (Ar) and consolidated into bulk materials by a powder extrusion process described below.

The powders were compacted at 230 °C in a vacuum to provide green compacts, 24 mm in diameter and 30 mm long, having relative densities of 75 to 85% and formed into billets for extrusion. The billets were extruded at 450 °C to produce extruded bars, about 6 mm in diameter, with an extrusion ratio of 15 and machined into test pieces for a tensile test. (measuring part: 3 mm in diameter and parallel parts: 15 mm). The test results are shown in Table 2.

Further test pieces were cut from the respective extruded bars for observation by TEM and average crystal grain size measurements were conducted. It was found that all of the test pieces had an average crystal grain size within the range of 5 to 60 »m and had a structure composed of a crystalline matrix containing uniformly dispersed intermetallic compounds of 20 to 50 nm.

**Table 2**

| Composition (at. %) | | Hv(DPN) | ^{σ}max^{(MPa)} | ε(%) |
|---|---|---|---|---|
| 1 | Al₈₇Ni₈Y₅ | 295 | 925 | 1.6 |
| 2 | Al₉₀Ni₅La₅ | 272 | 910 | 1.8 |
| 3 | Al₉₂Cu₄Ni₂Y₂ | 272 | 905 | 2.2 |
| 4 | Al₉₀Ni₆Zr₁Mm₃ | 287 | 945 | 2.4 |
| 5 | Al₉₀Ni₈Zr_{0.5}Mm_{1.5} | 293 | 941 | 2.2 |
| 6 | Al_{89.5}Ni₈Zr₁Fe_{0.5}Mm₁ | 285 | 937 | 1.9 |
| Remark: Hv(DPN): microVickers hardness ^{σ}max(MPa): ultimate tensile strength ε(%): Tensile elongation | | | | |

It was found that all of the test pieces had high strength and ductility and were superior as structural materials.

A further billet of Al₈₇Ni₆Mm₇ for extrusion was prepared in the same manner as described above and extruded at various temperatures to produce extruded bars. The changes in the tensile strength, hardness and tensile elongation were examined with respect to the changes in the average crystal grain size. The results are shown in FIG. 2.

As shown in FIG. 2, when the average crystal grain size was at least 0.1 »m, the tensile elongation was at least 0.5%. Whereas an average grain size of not more than 80 »m provided a high hardness of 200 (DPN), which was more than 2 times the hardness (Hv: 50 to 100 DPN) of a commercial aluminum-based alloy, coupled with a high strength level of at least 650 (MPa). A strength of at least 800 (MPa), a hardness of at least 230 (DPN) and an elongation of at least 1.2 (%) are the most desirable conditions for structural materials and it will be noted that these conditions can be satisfied within an average crystal grain size range of 22 to 60 »m.

As described above, the alloys of the present invention have a high degree of hardness, strength, wear resistance and heat resistance together with a superior toughness and are useful as highly reliable materials in structural components, etc.

## Claims

1. A high strength aluminum-based alloys having a composition consisting of the general formula (I)
AlₐM_{b}Ln_{c},
wherein:
M is at least one metal element selected from the group consisting of Co, Ni, and Cu;
Ln is at least one element selected from the group consisting of Y, rare earth elements and Mm (misch metal) which is a composite of rare earth elements; and
a, b and c are, in atomic percentage,
75 ≦ a ≦ 97, 0.5 ≦ b ≦ 15 and 0.5 ≦ c ≦ 10,
the alloy being composed of an aluminum matrix or an aluminum supersaturated solid solution matrix having an average crystal grain size of 0.1 to 80 »m and containing therein a uniform dispersion of metastable or stable phase particles composed of intermetallic compounds, which are formed between the host element (matrix element) and the above-mentioned alloying elements and/or between the alloying elements, the intermetallic compounds having an average particle size of 10 to 500 nm.

2. A high strength aluminum-based alloy having a composition consisting of the general formula (II)
AlₐM_{b}X_{d}Ln_{c},
wherein:
M is at least one metal element selected from the group consisting of Co, Ni, and Cu;
X is at least one metal element selected from the group consisting of V, Mn, Fe, Mo, Ti and Zr;
Ln is at least one element selected from the group consisting of Y, rare earth elements and Mm (misch metal) which is a composite of rare earth elements; and
a, b, c and d are, in atomic percentage,
75 ≦ a ≦ 97, 0.5 ≦ b ≦ 15, 0.5 ≦ c ≦ 10 and 0.5 ≦ d ≦ 3.5,
the alloy being composed of an aluminum matrix or an aluminum supersaturated solid solution matrix having an average crystal grain size of 0.1 to 80 »m and containing therein a uniform dispersion of metastable or stable phase particles composed of intermetallic compounds, which are formed between the host element (matrix element) and the above-mentioned alloying elements and/or between the alloying elements, the intermetallic compounds having an average particle size of 10 to 500 nm.

## Patentansprüche

1. Hochfeste Legierung auf Aluminiumbasis, die eine Zusammensetzung hat, welche aus der allgemeinen Formel (I) besteht
AlₐM_{b}Ln_{c},
worin:
M wenigstens ein metallisches Element, ausgewählt aus der aus Co, Ni und Cu bestehenden Gruppe, ist;
Ln wenigstens ein Element, ausgewählt aus der aus Y, Seltenerdelementen und Mm (Mischmetall), was ein Verbund aus Seltenerdelementen ist, bestehenden Gruppe, ist; und
a, b und c in Atomprozentsätzen sind:
75 ≦ a ≦97 , 0,5 ≦ b ≦ 15 , 0,5 ≦ c ≦ 10,
wobei die Legierung besteht aus einer Aluminiummatrix oder einer an Aluminium übersättigten festen Lösungsmatrix, die eine durchschnittliche Kristallkorngröße von 0,1 bis 80 »m hat und die hierin eine gleichförmige Dispersion von Teilchen einer metastabilen oder stabilen Phase enthält, zusammengesetzt aus intermetallischen Verbindungen, welche zwischen dem Wirtselement (Matrixelement) und den obengenannten Legierungselementen und oder zwischen den Legierungselementen gebildet sind, wobei die intermetallischen Verbindungen eine Durchschnittsteilchengröße von 10 bis 500 nm besitzen.

2. Hochfeste Legierung auf Aluminiumbasis, die eine Zusammensetzung hat, welche aus der allgemeinen Formel (II) besteht
AlₐM_{b}X_{d}Ln_{c},
worin:
M wenigstens ein metallisches Element, ausgewählt aus der aus Co, Ni und Cu bestehenden Gruppe, ist;
X wenigstens ein metallisches Element, ausgewählt aus der aus V, Mn, Fe, Mo, Ti und Zr bestehenden Gruppe, ist;
Ln wenigstens ein Element, ausgewählt aus der aus Y, Seltenerdelementen und Mm (Mischmetall), was ein Verbund aus Seltenerdelementen ist, bestehenden Gruppe, ist; und
a, b, c und d in Atomprozentsätzen sind:
75 ≦ a ≦97 , 0,5 ≦ b ≦ 15 , 0,5 ≦ c ≦ 10 und 0,5 ≦ d ≦ 3,5,
wobei die Legierung besteht aus einer Aluminiummatrix oder einer an Aluminium übersättigten festen Lösungsmatrix, die eine durchschnittliche Kristallkorngröße von 0,1 bis 00 »m hat und die hierin eine gleichförmige Dispersion von Teilchen einer metastabilen oder stabilen Phase enthält, zusammengesetzt aus intermetallischen Verbindungen, welche zwischen dem Wirtselement (Matrixelement) und den obengenannten Legierungselementen und oder zwischen den Legierungselementen gebildet sind, wobei die intermetallischen Verbindungen eine Durchschnittsteilchengröße von 10 bis 500 nm besitzen.

## Revendications

1. Alliage à base d'aluminium, à haute résistance, ayant une composition qui répond à la formule générale (I)
AlₐM_{b}Ln_{c} (I),
dans laquelle :
M est au moins un élément métallique choisi dans l'ensemble formé par Co, Ni et Cu;
Ln est au moins un élément choisi dans l'ensemble formé par Y, des éléments de terre rare et,
Mm (mischmetall) qui est un composite d'éléments de terre rare et,
a, b et c valent, en pourcentage atomique,
75 ≦ a ≦ 97; 0,5 ≦ b ≦ 15; 0,5 ≦ c ≦ 10 ,
l'alliage étant composé d'une matrice d'aluminium ou d'une matrice d'une solution solide sursaturée en aluminium ayant une taille moyenne des grains de cristal comprise entre 0,1 et 80 »m et contenant à l'intérieur une dispersion uniforme de particules de phase métastable ou stable constituée de composés intermétalliques, qui sont formés entre l'élément hôte (élément de la matrice) et l'alliage mentionné ci-dessus et/ou entre les éléments de l'alliage, les composés intermétalliques ayant une taille moyenne des particules comprise entre 10 et 500 nm.

2. Alliage à base d'aluminium, à haute résistance, ayant une composition qui répond à la formule générale (II)
AlₐM_{b}X_{d}Ln_{c} (II),
dans laquelle :
M est au moins un élément métallique choisi dans l'ensemble formé par Co, Ni et Cu;
X est au moins un élément métallique choisi dans l'ensemble formé par V, Mn, Fe, Mo, Ti et Zr ;
Ln est au moins un élément choisi dans l'ensemble formé par Y, des éléments de terre rare et
Mm (mischmetall) qui est un composite d'éléments de terre rare; et
a, b et c valent, en pourcentage atomique,
75 ≦ a ≦ 97; 0,5 ≦ b ≦ 15; 0,5 ≦ c ≦ 10 et 0,5 ≦ d ≦ 3,5,
l'alliage étant composé d'une matrice d'aluminium ou d'une matrice d'une solution solide sursaturée en aluminium ayant une taille moyenne des grains de cristal comprise entre 0,1 et 80 »m et contenant à l'intérieur une dispersion uniforme de particules de phase métastable ou stable constituée de composés intermétalliques, qui sont formés entre l'élément hôte (élément de la matrice) et l'alliage mentionné ci-dessus et/ou entre les éléments de l'alliage, les composés intermétalliques ayant une taille moyenne des particules comprise entre 10 et 500 nm.
